

## UNITED STATES PATENT OFFICE.

AMI REY, OF CALAIS, FRANCE.

## PROCESS FOR MANUFACTURE OF TILES.

No Drawing. Application filed April 25, 1927, Serial No. 186,587, and in France April 27, 1926.

The present invention relates to a process for the manufacture of tiles, sheets or covering material in iron or iron metals. It is a known fact that the great defect of iron 5 is its tendency to rust, and the present invention provides means for obviating all rusting, for giving the surfaces a determined color and agreeable aspect, and for diminishing the heat conductivity of the 10 metal.

In carrying my said process into effect, the objects such as tiles, covering sheets (plain or worked), fittings, gutters, pipes, ornaments and the like, are first cleaned and 15 then dipped into a bath of tar, pitch, bitumen, asphalt or the like; such substances are solid in the cold state and will not rust in air, and they are insoluble in water. The coating thus formed is quite adherent, and it 20 offers an effective protection of the iron against rusting. This treatment, which is known per se, is completed by the following treatment in which the invention essentially consists.

25 The aforesaid coating shows two defects. It has a more or less sticky nature and a displeasing color. The various colors which have been put in use upon the coating are found to adhere very imperfectly; they 30 will scale off, or are altered by the said coating which softens by heat and infiltrates into the color, thus forming spots and stains. In the present invention, I take advantage 35 of the agglutinating properties of the coating itself in order to fix the color. This latter consists of mineral substances which are hard, non-freezing, and unaffected by air or dampness, such as various stones or like mineral substances (granite, porphyry, 40 gneiss, basalt, marble, schist, waste bricks or tiles, natural sand and the like).

The said material is broken up, ground and sifted, and its degree of tenuity is regulated according to needs. A product which 45 traverses a No. 60 sieve but will not pass through a No. 70 will be suitable for most purposes.

50 The resulting color substance is heated in a suitable vessel at a temperature which is considerably above the melting point of the said coating. The coated objects are placed in contact with the hot color, upon which a certain pressure is exercised. When in contact with the hot color, the said coating will

melt and will enter between the grains of 55 the color by capillary action. The grains which are in immediate contact are entirely covered by the coating substance, and the succeeding grains are partially coated. Due to the agglutinating power of the coating 60 all the grains in contact therewith will be strongly held in place. The outer grains which are only partially covered will offer a free external face, so that the objects will have the desired color. Also, the resulting 65 surface has the advantage of presenting a dull color, and it has the appearance of the original stone; it will readily retain all pigments or coats which may be subsequently applied, and it gives the metal an added protection against mechanical and chemical 70 effects.

Before the objects are coated, they may be placed in a well-closed vessel and exposed to the action of the gas produced by the 75 dry distillation of coal, and when in contact with such gas, the objects will become heated and will be coated with an adherent film of carbon, which thus offers an additional protection. Furthermore, this gas, which is a 80 powerful reducing agent, will destroy all surface oxidation upon the iron.

The coloring substance, prepared as above stated, may be further applied by projecting it upon the objects coated with asphalt. 85

## I claim:

The herein-described process for the manufacture of tiles and the like, consisting in providing a sheet of metal of appropriate area, subjecting the metal in a well closed 90 vessel to the action of the gas produced by the dry distillation of coal, covering the treated metal with a coating which is insoluble in water and non-rusting, such as asphalt, and then applying a color substance 95 in the form of a finely ground mineral, with said color substance heated before application to a temperature above the melting point of the coating and subjecting the color coat to pressure to cause certain of the 100 grains of such coat to be wholly embedded in the first coating and certain of the grains to be partially embedded to leave the unembedded portions as a surface coloring layer for the tile. 105

In testimony whereof I affix my signature.

AMI REY.